

March 19, 1968

E. MEIER ET AL

3,374,163

## CELL FOR ELECTROLYSIS WITH MOLTEN SALT ELECTROLYTE

Filed Nov. 7, 1963



FIG 1



**FIG 2**

*Edwin Meier and  
Erich Schweizer  
INVENTOR*

BY *Bryant W. Brennan*,  
ATTORNEY

1

3,374,163

**CELL FOR ELECTROLYSIS WITH MOLTEN SALT ELECTROLYTE**

Edwin Meier and Erich Schweizer, Basel, Switzerland, assignor to Ciba Limited, Basel, Switzerland, a Swiss company

Filed Nov. 7, 1963, Ser. No. 322,106  
Claims priority, application Switzerland, Nov. 15, 1962,  
13,355/62  
3 Claims. (Cl. 204—246)

**ABSTRACT OF THE DISCLOSURE**

An electrolytic cell is provided for the manufacture of metals of the 4th, 5th and 6th sub-groups of the Periodic Table from the halide of the metal in a molten salt electrolyte. The cell has a hollow cylindrical anode and a rod-shaped cathode. The cathode is positioned within and coaxially aligned with the anode. The anode is characterized by having a plurality of annularly-arranged holes which extend downward from the inner wall of the anode to the outer wall of the anode. The cell has a downward-opening annular chamber positioned about the outer wall of the anode. In operation the cell is filled with a molten salt electrolyte to a level at which the surface of the electrolyte is slightly above the holes in the anode and in communication with the opening of the annular chamber. A vaporized metal halide is fed into the annular chamber from where it is introduced into the electrolyte. The holes in the anode assist the circulation of the electrolyte and facilitate the removal of the halide gases from the electrolyte in the cell.

Several electrolysis cells are known for the production of heavy metals by electrolysis by the continuous addition of a metal halide to a molten salt electrolyte. In some cases it has been proposed to supply the metal halide by a special supply feed directly to the cathode, or to introduce it into the melt bath through a hollow cathode. There are also known cells with a cylindrical anode and a rod-shaped cathode arranged coaxially thereto.

One of the main difficulties in the manufacture of heavy metals by electrolytic means is to discover conditions under which metal separates in as pure a state as possible.

Special difficulties are encountered, when the metal halide is added in vaporous state. The composition of the bath, the electrolysis temperature, the material of cathode, anode, vessel and diaphragm and the arrangement of the individual elements of the cell influence the electrolysis and, consequently, the quality and quantity of the metal separated. The arrangement and constitution of the cell is of particular importance. The present invention concerns this problem and provides a cell which makes it possible to manufacture especially pure metal.

It has been found pure metals of the 4th, 5th and 6th sub-group of the Periodic Table may be produced from the corresponding metal halide if the cell has the following features:

(1) The cell has no supply duct for the metal halide vapour into the melt, but only an arrangement whereby the metal halide is supplied to the surface of the melt. Thus, the metal halide is not introduced but flows on to the surface where it is absorbed by the molten salt bath on account of convection. The elimination of a duct submerged into the melt also eliminates the difficulty of having to introduce the metal halide under pressure. In addition, the elimination of the duct also prevents any additional contamination of the melt.

(2) An essential feature of the invention is that the condensing chamber for the metal halide, i.e., the place

2

where the halide is absorbed by the molten bath, is outside the zone of the electrolysis. According to the invention, it is arranged concentrically around electrolytic zone. This arrangement avoids losses of metal halide, such as occur during the condensation of the halide vapour in the electrolytic zone by discharge with the anode gas. Condensing chamber and electrolytic zone correspond to the principle of communicating vessels so that the level of the bath is the same in both parts of the cell.

(3) The cylindrically shaped anode contains in its upper portion, slightly below the level of the melt, several orifices in annular arrangement. These orifices produce a continuous circulation of the bath. In the inner part of the anode cylinder, the bath rises, flows through the orifices and down along the outside of the anode. In the inner part of the cylindrical anode, the halide is produced and the formed gas bubbles support the upward movement of the circulation in this zone.

(4) A special advantage of the arrangement of the invention is that no diaphragm is necessary. The supply of the metal halide vapour outside the electrolytic zone and the described circulation of the molten bath result in optimum conditions for the electrolysis so that no diaphragm is necessary.

The present invention relates to a cell for the electrolysis of halides of metals of the 4th, 5th and 6th sub-groups of the Periodic Table in a molten salt electrolyte, equipped with a feed duct for the vaporous metal halide and with a rod-shaped cathode, arranged coaxially within a cylindrical anode, characterized in that the condensing chamber for the metal halide is located outside the electrolytic zone, that the anode has preferably cylindrical holes in annular arrangement, slightly below the horizontal plane forming the upper defining line of the effective part of the rod cathode, and that there is arranged on the outside of the anode cylinder a downwardly open annular duct or channel, extending from the holes upwardly to above the upper defining plane of the effective portion of the rod cathode, above which horizontal plane there terminates at least one supply feed duct for the vaporous metal chloride into this annular channel.

FIG. 1 shows a diagrammatic arrangement of the cell, whilst FIG. 2 shows an embodiment of the cell.

FIG. 1 shows the cylindrical cathode, the hatched portion relating to the active part of the cathode, i.e., the part that is immersed in the bath. The level of the melt bath is at the same time the upper limit of the active part of the cathode rod. Below this limit there are the openings in the anode and, above, there is the non-immersed part of the annular channel, i.e., the so-called condensing chamber.

In FIG. 2 are shown the rod-shaped cathode 1, the cylindrical anode 2, the vessel 3, and a protective tube 4 over the cathode, forming at 5 the upper definition of the effective portion of the cathode. The level of the melt is shown at 6, a delivery duct at 7, and the outlet of the halogen gases formed at the anode at 8. Reference numeral 9 indicates a hinged cover. The vaporous metal halide enters at 10 and passes through 11 into the annular channel 12. The bath 13 circulates as indicated by the arrows. 14 is an orifice in the cylindrical anode. These orifices 14 are preferably of cylindrical shape, the longitudinal axis of the cylinder sloping downwardly toward the outside. This arrangement prevents the anode gas from being carried along into the condensing chamber. The supply feed duct 11 for the metal halide vapour terminates conveniently in the top of the annular channel 12.

Preferably a hollow cathode is used, with a water-cooled holder, and made of nickel. The cylindrical anode, as well as the vessel, are made of graphite. The top of the cell is closed so that access of foreign gases, such as air, is prevented.

The melts consist of mixtures of alkaline and alkaline earth halides, such as KCl, NaCl, KF, NaF, CaCl<sub>2</sub> or CaF<sub>2</sub>. Preferably mixtures are used which produce, after addition of the metal halide, stable double salts of the metal to be separated with the fluorides present in the bath.

The cell is suitable for producing titanium, zirconium, vanadium, chromium, molybdenum, tungsten, and especially tantalum and niobium. The metal halides supplied as vapours are especially metal chlorides, such as TiCl<sub>4</sub>, VCl<sub>5</sub>, VOCl<sub>3</sub>, NbCl<sub>5</sub>, TaCl<sub>5</sub> and WCl<sub>6</sub> and WOCl<sub>4</sub>.

#### EXAMPLE 1

In an electrolytic cell according to FIG. 2, about 40 kg. of a salt mixture, consisting of 40% sodium chloride, 30% potassium chloride and 30% potassium fluoride, are molten at about 800° C. Into this melt, about 7 kg. tantalum pentachloride are added as vapour by convection through conduit 11 and annular channel 12. Electrolysis is effected at a bath temperature of 800° C. to 900° C. with 1500 amps. In order to maintain the concentration of tantalum chloride in the melt, 3.6 kg. TaCl<sub>5</sub> are introduced in the course of one hour. After one hour, the separated metal is removed from the cell and further electrolysis is carried out with a second cathode. 1710 grams of tantalum are separated during this time. The yield—related to TaCl<sub>5</sub>—is 95% and the mean current yield is 83%. The metal produced has a uniform, metallic appearance and consists of dendrites of 100 to 500 microns. An analysis shows the following impurities:

|            | Percent, below |
|------------|----------------|
| Carbon     | 0.02           |
| Oxygen     | 0.02           |
| Hydrogen   | 0.002          |
| Nitrogen   | 0.005          |
| Silicon    | 0.001          |
| Tungsten   | 0.003          |
| Molybdenum | 0.001          |
| Niobium    | 0.005          |
| Chromium   | 0.005          |
| Nickel     | 0.01           |
| Iron       | 0.005          |
| Titanium   | 0.001          |

#### EXAMPLE 2

A cell as shown in FIG. 2 is used. 2.5 kg. of titanium tetrachloride are added as vapour through annular channel 12 and absorbed in 35 kg. of a basic melt consisting of 40 percent by weight of sodium chloride, 40 percent by weight of potassium chloride and 20 percent by weight of potassium fluoride; electrolysis is carried out for 1 hour at 1000 amps. and at a bath temperature of 800° C. A further 2.5 kg. of titanium tetrachloride are added as vapour during electrolysis. The separated metal on the cathode is cooled in an atmosphere of argon; after washing, the weight of the metal is 327 grams which corresponds to a current yield of 72.6% and a metal yield of 89%. An analysis shows the following values:

|            | Percent, below |
|------------|----------------|
| Carbon     | 0.02           |
| Oxygen     | 0.02           |
| Hydrogen   | 0.005          |
| Silicon    | 0.001          |
| Molybdenum | 0.001          |
| Chromium   | 0.01           |
| Nickel     | 0.03           |
| Iron       | 0.02           |
| Tungsten   | 0.003          |

#### EXAMPLE 3

In each case a cell as shown in FIG. 2 is used.

(a) 6 kg. of tungsten hexachloride are added as vapour into a basic melt of the same composition as described in Example 2 and electrolyzed as described in Example 2.

The washed metal weighs 784 grams. The current yield is 68.4%, the metal yield 83%.

(b) 4 kg. of tungsten oxychloride are added as vapour into the above melt and subjected to electrolysis at 1000 amps for 1 hour to yield 724 grams of metal. The current yield is 63%, the metal yield 85%.

An analysis shows the following values:

|            | Percent, below |
|------------|----------------|
| Carbon     | 0.03           |
| Oxygen     | 0.03           |
| Hydrogen   | 0.005          |
| Silicon    | 0.001          |
| Molybdenum | 0.001          |
| Chromium   | 0.01           |
| Nickel     | 0.03           |
| Iron       | 0.02           |
| Titanium   | 0.001          |

#### EXAMPLE 4

20 A cell as shown in FIG. 2 is used. A total of 3 kg. of niobium pentachloride is added as vapour through annular channel 12 into a basic melt of 17.1 kg. of sodium chloride, 9.8 kg. of potassium chloride and 13.0 kg. of potassium fluoride. The bath temperature is 900° C. Electrolysis is carried out for 1 hour with 1200 amps. The weight of the metal separated during this time amounts, after washing, to 310 grams, which corresponds to a current yield of 37.2%. After analysing the niobium remaining in the melt, a material yield of 89.5% was found.

30 An analysis shows the following values:

|            | Percent, below |
|------------|----------------|
| Carbon     | 0.03           |
| Oxygen     | 0.03           |
| Hydrogen   | 0.005          |
| Silicon    | 0.001          |
| Tungsten   | 0.003          |
| Molybdenum | 0.001          |
| Tantalum   | 0.01           |
| Chromium   | 0.01           |
| Nickel     | 0.03           |
| Iron       | 0.02           |
| Titanium   | 0.001          |

What is claimed is:

1. Cell for the electrolysis of halides of metal of the 4th, 5th and 6th sub-groups of the Periodic System, in a molten salt electrolyte, having a supply feed for the vaporous metal halide and a rod-shaped cathode, arranged coaxially within a cylindrical anode, characterized in that the condensing chamber for the metal halides is outside the electrolytic zone; that the anode has cylindrical holes in annular arrangement slightly below the horizontal plane forming the upper defining line of the effective part of the rod cathode the remainder of said anode being non-foraminous, said holes having a cylindrical shape and their longitudinal axis sloping downwardly and outwardly, and that a downwardly open annular channel is arranged on the outside of the cylindrical anode, extending from said holes upwardly to above the horizontal plane forming the upper definition of the effective part of the rod cathode, above which horizontal plane there terminates at least one supply duct for the vaporous metal halide in this annular channel.

2. A cell as claimed in claim 1, characterized in that the supply duct for the metal halide terminates in the top of the annular channel.

3. An electrolytic cell for the manufacture of the metals of the 4th, 5th and 6th sub-groups of the Periodic Chart from a halide of said metals using a molten salt electrolyte, said electrolytic cell comprising in combination: a rod-shaped cathode, a hollow cylindrical anode having inner and outer walls, a downward opening annular chamber and a supply duct; said cathode being positioned within and coaxially aligned with said anode, said anode being adapted to be immersed in said electrolyte to a predetermined level and having a plurality of cylindrical

downward-extending apertures from the inner wall to the outer wall arranged annularly about said anode at a position which is only slightly below the surface of the electrolyte when the anode is emersed to said predetermined level, the remainder of said anode being non-foraminous said annular chamber being positioned about the outer wall of the anode so that it is in communication with the surface of the electrolyte when the anode is emersed to the predetermined level, and said supply duct being in communication with the annular chamber and adapted to feed said metal halide, in vaporized form, to the annular chamber.

## References Cited

## UNITED STATES PATENTS

|           |         |              |       |           |
|-----------|---------|--------------|-------|-----------|
| 2,898,276 | 8/1959  | Snow         | ----- | 204-246 X |
| 2,908,619 | 10/1959 | Barnett      | ----- | 204-246 X |
| 3,079,324 | 2/1963  | Allen et al. | ----- | 204-246   |

HOWARD S. WILLIAMS, *Primary Examiner.*

JOHN H. MACK, *Examiner.*

10 D. R. VALENTINE, *Assistant Examiner.*